

[54] GAME BALL

[75] Inventor: **Jesse H. Heald, Jr.**, Tullahoma, Tenn.[73] Assignee: **Lannom Manufacturing Company, Inc.**, Tullahoma, Tenn.[22] Filed: **Feb. 20, 1976**[21] Appl. No.: **659,705****Related U.S. Application Data**

[63] Continuation of Ser. No. 487,203, July 10, 1974, abandoned.

[52] **U.S. Cl.** ..... 273/60 R; 273/DIG. 8; 264/299[51] **Int. Cl.<sup>2</sup>** ..... A63B 37/00[58] **Field of Search** ..... 273/60, DIG. 8, 58 J, 273/58 G, 58 H, 218, 58 A, 26 R[56] **References Cited**

## UNITED STATES PATENTS

2,081,531 5/1937 Fegan ..... 273/60 R  
2,138,004 11/1938 Grau ..... 273/60 R

|           |         |                  |            |
|-----------|---------|------------------|------------|
| 3,069,170 | 12/1962 | Dillon.....      | 273/60 B   |
| 3,185,476 | 5/1965  | Fechner.....     | 273/DIG. 8 |
| 3,518,786 | 7/1970  | Holtvoigt.....   | 273/DIG. 8 |
| 3,644,168 | 2/1972  | Bonk et al. .... | 273/DIG. 8 |
| 3,940,145 | 2/1976  | Gentiluomo.....  | 273/218    |

*Primary Examiner*—George J. Marlo  
*Attorney, Agent, or Firm*—Mason, Fenwick & Lawrence

[57]

**ABSTRACT**

A ball is disclosed formed with a spherical core of polyurethane foam covered with a thin winding of cotton yarn and with a hand stitched outer cover; the ball is formed in a mold by providing a polymeric isocyanate with a mixture of water and a polyol crosslinking catalyst with the ratio between the isocyanate and the mixture of the catalyst and the water being variable to provide a ball of desired resilience and density so that the ball formed by the method can duplicate such characteristics as found in conventional baseballs and softballs.

**15 Claims, 6 Drawing Figures**



Fig-3



Fig-5



Fig-6

## GAME BALL

## PRIOR RELATED APPLICATION

This application is a continuation of prior application Ser. No. 487,203, filed July 10, 1974, now abandoned.

## BACKGROUND OF THE INVENTION

This invention is in the field of balls per se and the fabrication of balls. More specifically, the subject invention is in the field of baseballs and softballs and is particularly directed to a ball construction and method providing either a baseball, softball or similar ball having desired characteristics essentially identical to prior conventional balls, but having uniformity of construction, cost and durability advantages over prior known conventional balls.

Conventional baseballs are formed with a cork and rubber center over which winding of wool and cotton are provided with the entire assembly being maintained in a handsewn leather cover in the well-known figure eight pattern. The weight of the ball is determined by the density of the separate materials used in the ball and the tension of the wool yarn windings. Normally, the winding of cotton thread merely serves to provide a smooth surface onto which the leather cover is sewn. The weight of the baseball is determined by the density of the separate material employed in the ball and the tension of the wool windings. Consequently, the ball weight and resilience are related and cannot be controlled or varied independently of each other. The vast majority of baseballs used in organized league play such as in highschool, college, professional youth leagues and the like are formed in this traditional manner.

Softballs, on the other hand, come in a substantial number of different sizes but with all of the balls being of the same basic type construction. This commonly employed construction includes a core of cork or kapok. The core is wound with cotton or synthetic yarn over which a handstitched leather cover in the traditional figure eight pattern is provided. When a cork core is employed, it is normally mixed with a suitable binder before molding to add strength to the finished core portion. The weight of the softball is determined by the weight of the separate materials used and the resiliency is determined primarily by the cork or kapok core. As in the case with the conventional baseball, the weight and resiliency of the ball cannot be controlled independently of each other.

The materials employed in the conventional baseballs and softballs are relatively expensive with additional costs resulting from the substantial amount of hand labor required for the fabrication of such balls.

Therefore, it is the primary object of this invention to provide a new and improved ball construction as well as a new and improved method of ball fabrication.

## SUMMARY OF THE INVENTION

Achievement of the object of the invention is enabled through the employment of a hollow spherical mold for forming the core of the ball of polyurethane foam produced by the reaction of three separate liquid components. These components are introduced into the mold in desired ratios to provide desired resiliency and rebound characteristics as well as a desired weight. The components comprise isocyanate and a mixture of a polyol crosslinking catalyst and water. The ratio of the

catalyst to the isocyanate determines the degree of polymerization and crosslinking of polymers which in turn determines the resiliency. The blowing agent is the water in the mixture which reacts with the isocyanate

5 to produce carbon dioxide to cause foam expansion of the components during the polymerization process. Once the desired ratio of catalyst to the isocyanate has been determined to produce the desired resilience, the 10 amount of blowing agent is determined to produce the desired density and weight for the particular ball being constructed. Consequently, the resilience and weight are controlled independently of each other.

15 After formation of the core of the polyurethane foam, the core is then coated with a winding of thin cotton yarn over which a leather or synthetic cover is provided in a conventional manner. For example, if a baseball is being provided, a horsehide is hand sewn about the core and the intermediate winding of cotton yarn to provide a resultant ball having the exact same 20 appearance, weight and resilience as a conventional baseball. Similarly, a ball having the exact same resilience, weight and appearance as any of the various types of conventional softballs can also be provided through employment of the inventive method.

25 A better understanding of the subject invention will be achieved when the following written description is considered in conjunction with the appended drawings.

## DESCRIPTION OF THE DRAWINGS

30 FIG. 1 is an exploded perspective illustrating open mold means employed in practice of the preferred embodiment illustrating an initial step in the inventive method;

35 FIG. 2 is a perspective view of the mold means in a closed condition;

FIG. 3 is a sectional view taken along lines 3—3 of FIG. 2;

40 FIG. 4 is a perspective view illustrating separate components of an incompletely fabricated ball embodying the present invention;

FIG. 5 is a perspective view illustrating a subsequent step in the assembly of the inventive ball with portions removed to illustrate the structure thereof; and

45 FIG. 6 is a perspective view of another embodiment of the inventive ball with portions removed to illustrate the internal construction of the ball.

## DESCRIPTION OF THE PREFERRED EMBODIMENT

50 Attention is initially invited to FIG. 1 of the drawings which illustrates a mold member comprising an upper mold portion 10 and a lower mold portion 12 which cooperate when placed together in the position illustrated in FIG. 2 to define a spherical cavity 14 which communicates with a vent 20 in the upper mold member 10.

55 The mold members 10 and 12 are employed for producing ball members as disclosed in FIGS. 4-6. Each of the ball members is formed with a spherical core portion 22 of polyurethane foam having a diameter equal to at least 90% of the desired finished ball diameter. A cover 24 of horsehide or other material is sewn over and about the spherical core portion 22 with the cover normally being in a figure eight design as in the case 60 with a conventional baseball or softball. The core portion 22 can have the cover 24 directly applied about its exterior surface as when forming a softball as shown in FIG. 5 or an intermediate layer of cotton or other yarn

65

26 can be provided over the surface of the spherical core member prior to the application of the cover 24 to provide a baseball as shown in FIG. 6.

The core is fabricated by placing carefully measured amounts of polymeric isocyanate and a mixture of a catalyst and a blowing agent in the mold members so that the reaction of the constituents placed in the mold provides a resultant spherical core member as shown in FIG. 3. The blowing agent is water which reacts with the isocyanate to produce carbon dioxide gas to cause expansion and foaming of the mixture during polymerization. Normally, the water and the polyol catalyst are mixed together prior to mixing with the isocyanate. Consequently, the resulting ball weight and resilience can be controlled independently by controlling the ratio of the catalyst and blowing agent to the quantity of isocyanate.

The manner in which the subject invention is practiced will be made more apparent by consideration of the following specific examples of methods employed in the fabrication of balls having different characteristics. In a first example, commercially available isocyanate sold under the trademark FLEXIPOL and designated FP123 in its catalogue by Flexible Products Company of Marietta, Georgia was mixed in the mold with a mixture of catalyst and blowing agent (water) with ratio of the isocyanate to the mixture of catalyst and blowing agent being 0.418. The total compound weight was 125 grams and the mold was dimensioned to provide a core of slightly less than standard softball size. The components were permitted to cure in the mold for approximately 10 minutes and the core was then removed and covered with an intermediate thin cotton yarn layer over which a cowhide cover was applied. The resultant ball had a rebound characteristic of 30%. In other words, the ball would bounce to a height equal to 30% of the height from which it was dropped.

In a second example, commercially available isocyanate also sold under the trademark FLEXIPOL by Flexible Products Company but designated FP124A in its catalogue was mixed in the mold with a mixture of catalyst and blowing agent in a ratio of the isocyanate to the mixture of the catalyst and blowing agent of 0.396 with the total weight of the components being 125 grams. The core was slightly less than the finished size of the standard softball and the core was covered with cotton yarn and a cowhide cover with the resultant ball being of standard softball size and having a rebound percentage of 23%. The isocyanate employed in this example has a shorter molecular length than does the isocyanate of the previous example.

In a third example, the components were the same as in the second example, but with the ratio of the isocyanate to the mixture of the catalyst and blowing agent being 0.375 and the resultant ball having a percent rebound of 21.5%.

In a fourth example, the constituents were exactly the same as in the second example and the ball was formed in exactly the same manner with the exception that the ratio of the isocyanate to the mixture of catalyst and blowing agent was 0.361. The resultant ball had a rebound percentage of 20.5%.

In all of the foregoing examples, the softball core had a circumference of 11.25 inches and a weight of 125 grams. The finished softball weighed 182 grams.

By changing the catalyst and blowing agent from that of the first example to that of the second, third and

fourth examples, the resiliency of the ball was reduced with no change in weight. Further changes in the resiliency were effected between the balls formed in the second, third and fourth examples by merely changing the ratio of the isocyanate to the mixture of the blowing agent and catalyst with the balls retaining the same weight. Consequently, it will be apparent that the increase in the amount of catalyst serves to reduce the resilience of the ball and vice versa. This is true because increased amounts of catalyst terminate the polymerization process more quickly than is the case with reduced quantities of catalyst so that the crosslinking of the polymers is reduced to consequently reduce the resilience.

Compression tests performed upon the inventive cores indicate that the polyurethane core member has a greater ability to recover from compression than do conventional cork softball cores. Moreover, the polyurethane core members have a greater strength than do cork cores which tend to crumble and crack after the core has been compressed by more than one-half their diameter. For example, a cork core will recover only 76% of its initial diameter after being subjected to maximum deflection while a polyurethane core will recover 93% of its initial diameter.

Additionally, while the foregoing examples have discussed the provision of a ball having a polyurethane core, it should be understood that a one-piece ball can be produced in the mold member with a stitch pattern being applied to the internal surface of the mold. In such cases, the mold will be maintained at 100° to 120°F during the molding process for approximately 10 to 15 minutes. The mold will then be open and the ball removed to provide a completed ball in which the outer skin surface of the polyurethane constitutes the cover.

It should be understood that the spirit and scope of this invention is not limited to the specifically discussed examples, and is to be limited solely by the appended claims.

I claim:

1. A composite ball having the appearance, physical characteristics and dimensions of a conventional baseball including a cork and rubber center, yarn windings, and a leather cover comprising a spherical core member formed of flexible and resilient molded polyurethane foam and a cover portion comprising a leather member stitched over and enclosing said core member wherein said core member is formed of polyurethane foam of such density and resilience as to give said composite ball essentially the same rebound qualities, hardness, size, feel and sound as said conventional baseball so as to be usable in organized league play of baseball under the rules of baseball.

2. The composite ball of claim 1 wherein the diameter of said core member is equal to at least 90% of the diameter of the finished composite ball.

3. A composite ball having the appearance, physical characteristics and dimensions of a conventional softball including a core of cork or kapok, yarn windings, and a leather cover comprising a spherical core member formed of flexible and resilient molded polyurethane foam and a leather cover portion enclosing and stitched over said core portion wherein said core portion is formed of polyurethane foam of such density and resilience as to give said composite ball essentially the same rebound weight, hardness, size, feel and sound qualities as said conventional softball so as to be usable in organized league play of softball.

4. The composite ball of claim 3 wherein the diameter of said core member is equal to at least 90% of the diameter of the finished composite ball.

5. The composite ball of claim 3 wherein said spherical core member is formed from a mixture of isocyanate and a mixture of catalyst and blowing agent.

6. The composite ball of claim 5 in which the ratio of the isocyanate to the mixture of catalyst and blowing agent is approximately 0.418 and said composite ball has a rebound percentage of 30%.

7. The composite ball of claim 5 in which the ratio of the isocyanate to the mixture of catalyst and blowing agent is approximately 0.396 and said composite ball has a rebound percentage of 23%.

8. The composite ball of claim 5 in which the ratio of isocyanate to the mixture of catalyst and blowing agent is 0.375 and said composite ball has a percentage rebound of 21.5%.

9. The composite ball of claim 5 in which the ratio of isocyanate to the mixture of catalyst and blowing agent is 0.361 and said ball has a rebound percentage of 20.5%.

10. The invention of claim 5 in which said spherical core member has a circumference of approximately 11.25 inches and a weight of approximately 125 grams.

11. The invention of claim 10 in which the ratio of the isocyanate to the mixture of catalyst and blowing agent is approximately 0.418 and said composite ball has a rebound percentage of 30%.

12. The invention of claim 10 in which the ratio of the isocyanate to the mixture of catalyst and blowing agent is approximately 0.396 and said composite ball has a rebound percentage of 23%.

13. The invention of claim 10 in which the ratio of isocyanate to the mixture of catalyst and blowing agent is 0.375 and said composite ball has a percentage rebound of 21.5%.

14. The invention of claim 10 in which the ratio of isocyanate to the mixture of catalyst and blowing agent is 0.361 and said ball has a rebound percentage of 20.5%.

15. The composite ball of claim 10 in which the total weight of said composite ball is 182 grams.

\* \* \* \* \*

25

30

35

40

45

50

55

60

65

**REEXAMINATION CERTIFICATE (1244th)**  
**United States Patent [19]** [11] B1 3,976,295  
**Heald, Jr.** [45] Certificate Issued Apr. 10, 1990

**[54] GAME BALL**

[75] Inventor: **Jesse H. Heald, Jr., Tullahoma, Tenn.**

[73] Assignee: **Lannom Manufacturing Co. Inc.**

**Reexamination Request:**  
No. 90/001,755, Apr. 20, 1989

**Reexamination Certificate for:**

Patent No.: **3,976,295**  
Issued: **Aug. 24, 1976**  
Appl. No.: **659,705**  
Filed: **Feb. 20, 1976**

**Related U.S. Application Data**

- [63] Continuation of Ser. No. 487,203, Jul. 10, 1974, abandoned.  
[51] Int. Cl.<sup>4</sup> ..... **A63B 37/00**  
[52] U.S. Cl. ..... **273/60 R; 273/DIG. 8;  
264/299**

**[56] References Cited**

**U.S. PATENT DOCUMENTS**

- 2,743,931 5/1956 Pooley et al. ..... 273/199  
2,753,599 7/1956 Pietraszek et al. ..... 18/47.5

3,647,229 3/1972 Holley ..... 273/235

**FOREIGN PATENT DOCUMENTS**

632220 12/1951 Canada .

**OTHER PUBLICATIONS**

Dr. J. Adin Mann, Jr., Resume.  
The Flexible Polyurethane Foam Handbook, Dow Chemical, U.S.A.  
Modern Plastics Encyclopedia, 1966, pp. 177-180.  
Plastic Foams: The Physics and Chemistry of Product Performance and Process Technology, vol. II, pp. 67-81.

*Primary Examiner*—Maurice J. Welsh

**[57] ABSTRACT**

A ball is disclosed formed with a spherical core of polyurethane foam covered with a thin winding of cotton yarn and with a hand stitched outer cover; the ball is formed in a mold by providing a polymeric isocyanate with a mixture of water and a polyol crosslinking catalyst with the ratio between the isocyanate and the mixture of the catalyst and the water being variable to provide a ball of desired resilience and density so that the ball formed by the method can duplicate such characteristics as found in conventional baseballs and soft-balls.

**REEXAMINATION CERTIFICATE  
ISSUED UNDER 35 U.S.C. 307**

NO AMENDMENTS HAVE BEEN MADE TO  
THE PATENT

AS A RESULT OF REEXAMINATION, IT HAS  
BEEN DETERMINED THAT:

5 The patentability of claims 1-15 is confirmed.

\* \* \* \* \*

10

15

20

25

30

35

40

45

50

55

60

65